# EUROPEAN PATENT SPECIFICATION

(11) **EP 0 088 192 B1**
(45) Date of publication and mention of the grant of the patent: **05.11.1986**
(21) Application number: 82306911.7
(22) Date of filing: 23.12.1982
(51) Int. Cl.: C25D 3/06

(54) **Control of anode gas evolution in trivalent chromium plating bath**
Überwachung von Anodengasentwicklung in einem dreiwertigen Chromplattierungsbad
Contrôle d'évolution de gaz d'anode dans un bain de placage à base de chrome trivalent

(30) Priority: 05.03.1982 US 354999
(43) Date of publication of application: 14.09.1983
(73) Proprietor: M & T CHEMICALS, INC., Woodbridge, New Jersey 07095 (US)
(72) Inventor: Seyb, Edgar John, Jr., Freehold New Jersey 07728 (US); Brown, Laurence Arthur, Carteret New Jersey 07008 (US)
(74) Representative: Ellis, John Clifford H.

## Description

This invention relates to a process for the electroplating of chromium from aqueous plating baths and more in particular it relates to the production of chromium electrodeposits from a trivalent chromium plating bath. It also relates to a novel trivalent chromium plating bath.

Chromium has been electrodeposited from trivalent plating baths primarily for decorative purposes. Generally it has not been utilized for functional chromium plating since the adhesion to the substrate has been poorer than the adhesion of chromium elecroplates produced from hexavalent chromium plating baths.

The adhesion produced in trivalent chromium plating operations had been sufficient for decorative purposes and provides several advantages as compared to plating from hexavalent chromium plating baths. These include:
1. Higher coverage and freedom from burn at high current densities;
2. Good coverage at low current densities;
3. Reduced sensitivity to current breaks;
4. Fewer problems with waste disposal.

However, in addition to the aforementioned adhesion difficulties, there are several other problems attendant to the use of trivalent chromium plating baths. First, the deposit quality tends to deteriorate rapidly due to the formation of even a few parts per million of hexavalent chromium at the anode. The hexavalent chromium is very detrimental to the quality of the chromium electroplate since black streaks tend to be produced, thereby marring the appearance of the plate.

Further, conventional trivgient chromium.plating bath compositions usually include sulfate ions as conductivity anions. Inasmuch as the generally utilized anodes are graphite anodes, oxygen is released during plating operations and can attack the anode causing erosion and the release of carbon particles into the bath. The resultant carbon particles tend to become included in the chromium electrodeposit thereby producing defects in the plate.

It has been suggested that the incorporation of salts containing a halogen anion in the bath will suppress the production of oxygen and thereby yield a better quality electrodeposit with longer bath life. For example, U.S. Patent No. 3,833,485 suggests that the utilization of relatively high concentrations (0.05 M to 4 M) of either chloride ions or bromide ions in the bath will reduce anode erosion. The minimum useful concentrations are stated to be 0.01 M.

Generally, due to cost factors, chloride ion has been the halogen ion of choice. However, when utilizing effective levels of chloride ions in such plating baths, noxious chlorine gas is given off at the anode.

It has now been found that the use of the combination of low concentrations of bromide ion in conjunction with a nitrogen containing cation in chloride-containing trivalent chromium plating baths inhibits the evolution of chlorine, or other noxious gases, at the anode during plating operations.

In accordance with the present invention, chromium is electroplated from a trivalent chromium plating bath which include a combination of a substantial amount of chloride ion, a nitrogen containing cation and from 0.004 mole per liter to 0.008 mole per liter of bromide ion, thereby suppressing the formation of chlorine gas and hexavalent chromium at the anode during the electroplating process. The optimum balance between cost and effectiveness is achieved in the above range of bromide ion. The plating behavior of the bath has been found to be independent of the bromide concentration, and this formation represents an appreciable cost saving over prior art.

The trivalent chromium electroplating bath and process of this invention are useful to provide decorative bright chromium electrodeposits. These electrodeposits may be produced on any type of metallic substrate material, but commercially, ferrous metal substrates are generally utilized. While not essential, it is standard commercial practice to first form an electroplate of bright nickel on the substrate material. Alternatively, bright electrodeposits of cobalt, nickel-iron alloy, cobalt-iron alloy, nickel-cobalt-iron alloy or copper could be utilized as the initial coating material for the substrate.

The nickel electrodeposit serves to provide a smooth surface onto which the chromium will be deposited. If this surface is not provided, it is believed to be unlikely that the thin chromium deposit would be sufficiently bright for consumer acceptance. The nickel electrodeposit also serves to provide corrosion resistance to the substrate material which is particularly valuable for outdoor usage of the manufactured item. The nickel electrodeposit is not to be confused with a nickel "strike" but is actually a substantial deposit of material. It is general commercial practice to provide a nickel deposit of about 0.1 mil (2.5 pm) to about 0.5 mil (13 pm) for indoor utilization and from about 1.0 mil (25 pm) to about 1.5 mils (38 um) for outdoor utilization.

The trivalent chromium plating bath of this invention is conventional with the exception of the nitrogen-containing cation or substance yielding the nitrogen-containing cation in conjunction with a bromide ion content of 0.004 to 0.008 mole per liter. Similarly the process details follow normal commercial practice. Details of each may be found in the aforementioned U.S. Patent No. 3,833,485, the relevant portions of which are incorporated herein by reference. The bath and process parameters are discussed hereinafter.

It should be noted that U.S. Patent No. 3,833,485 discloses the use of a halogen, either chlorine or bromine to preclude oxygen liberation at the anode. By way of contrast, in the instant invention, chlorine and bromine are not optional alternatives, but rather are both essential additives. The chlorine is an essential conductivity anion and prevents hexavalent chromium formation at the anode. The presence of hexavalent chromium in concentrations as low as several parts per million can poison the bath. The bromine is critical in order to preclude chlorine generation at the carbon anode.

US-A-4093521 describes a trivalent chromium electroplating bath which consists essentially of an acidic aqueous solution of trivalent chromium, a carboxylate selected from formate, acetate and mixtures thereof, a bromide and ammonium, wherein certain Fe and/or Ni amounts are maintained. The concentration of bromide is preferably above 0.01 molar, particularly from 0.05 to 0.3 molar, best results being said to be obtained when the concentration of bromide is greater than 0.1 molar. In the plating bath of this publication, chloride is an optional and preferable addition.

US―A―4167460 describes an aqueous acidic trivalent chromium electroplating solution containing a complexing agent, such as ammonium formate or ammonium acetate, a reducing agent, e.g. bromide in concentrations of from about 0.01 up to a.bout 4 molar, and a controlled amount of organic mono- di- ortri- ester phosphates. Chlorides may be present in the bath.

Generally any water soluble salt wherein chromium is present in the trivalent state may be utilized in the plating bath. Generally chromic chloride, chromic sulfate or a mixture thereof is utilized due to their low cost and ready availability.

We have found it convenient to utilize a material known as "chromium tanning salt". This is a commonly available form of chromic sulfate, the formula of which is often written Cr(OH)S0₄.xH₂0. However, it is believed to be actually a mixture of hydrated basic chromic sulfates, the exact composition of which will be dependent on the pH of the solution from which it was crystallized.

The chromium salt may be present over a relatively wide range of concentrations. Generally the chromium ion may be present in the range of from about 0.001 mole per liter to the limit of solubility of the chromium salt. The preferred range is from about 0.01 mole per liter to about 1.0 moles per liter. It is general commercial practice to utilize an initial chromium ion concentration at about the middle of the preferred range. This will ensure that the concentration does not drop during the plating process to a level so low that there may be some burn to the plated item. Further, it is commercially undesirable to have too high a chromium ion concentration as one can encounter waste disposal problems.

The bath will, of course, include substantial amounts of various salts to greatly increase the electrical conductivity of the bath. These salts and their constituent ions are generally considered to be salts other than the chromium salt. It is general practice to utilize from about 2 moles per liter to about 6 moles per liter of total conductivity salt. A commercially preferred range is from about 3.5M to about 5.5M. The terms conductivity cation and conductivity anion refer to the cations and anions respectively constituting the conductivity salt. The conductivity anion includes the anionic species which is introduced with the chromium cation.

Generally, but not necessarily, an important conductivity anion is sulfate ion. Sulfate ion is, of course, present whenever chromic sulfate is utilized as a source of chromium ions. When additional sulfate ion is deemed to be desirable, it may be introduced in any water soluble form. It may be most convenient to introduce it in the form of sulfuric acid, which may aid in pH adjustment, or as ammonium sulfate for reasons discussed below. In any event, the use of sulfate ion in the plating bath is not essential, but is particularly convenient. In its broadest range, the sulfate ion may comprise any amount up to about 90% (all percentages herein on a mole basis) of the total conductivity anion in the bath.

The presence of chloride ion is essential for satisfactory chromium plating from the instant trivalent chromium plating bath. Preferably it should be present in an amount of at least 5% of the total conductivity anion present in the plating bath. For certain uses, it may even constitute all of the conductivity anion present in the bath. Most preferably chloride ion is present in an amount which constitutes from about 10% to about 90% of the total conductivity anion present in the plating bath. Commercially, it is generally utilized at a concentration of 50% or higher.

The chloride ion may be introduced in any convenient water soluble form. It is conveniently introduced as hydrochloric acid, ammonium chloride, an alkali metal chloride or mixtures thereof. Of course, it may be also added as chromic chloride.

It is highly desirable that the nitrogen containing cation be present in an amount equal to at least 5% of the total conductivity cation present in the bath. Preferably such cation is present in an amount equal to about 20% to about 90% of the total conductivity cation. It is most convenient to add the nitrogen containing cation to the bath in the form of an ammonium salt, such as the sulfate or chloride as described above. However, it may also be introduced in other forms, such as urea, hydrazine, hydroxylamine, or a variety of other amine materials which are generally added in the form of the sulfate or hydrochloride.

While it is believed that the nitrogen containing cation itself may be oxidized at the anode, this process is not sufficient to prevent the production of chlorine gas at the anode. However, it is believed that the nitrogen containing cation is able to reduce the bromine produced at the anode to regenerate bromide ion. Thus, while the nitrogen containing cation is consumed during the plating operations, the bromide ion will not be consumed, it is critical that the nitrogen containing cation be present if the bromide is to function at the very low levels utilized in this invention.

The bromide ion of this invention is present in an amount ranging from 0.004 mole per liter to 0.008 mole per liter. Commercially it will be generally utilized in amounts of about 0.0075 mole per liter to ensure that there is at least the optimum concentration present throughout the bath. If there is insufficient bromide ion present, one does not obtain a sufficiently high level of anode gas suppression to have any commercial viability. The utilization of too high a level of bromide ion provides no greater effect and is not economically viable from a commercial standpoint as bromide salts are generally quite expensive.

The bromide ion may be added conveniently in any manner similar to the addition of the chloride ion.

Generally, boric acid or a borate salt or both will also be included in the plating baths of this invention. The presence of the boric acid and/or borate serves to assist in pH control of the system. These materials are generally utilized in a total amount of about 0.1 to about 1 mole per liter, measured as boron.

Further, it will generally be advantageous to include a formate salt in the bath to improve the appearance of the plated product arid provide greater covering power for the bath. Formate ions are generally utilized in the range of about 0.1 mole per liter to about 1.5 moles per liter. The formate may need to be replenished from time to time as it tends to be oxidized at the anode.

Acetate ions may also optionally be incorporated into the bath to assist in preventing the formation of hexavalent chromium.

Of course, other conventional additives may be utilized in the instant trivalent chromium plating baths.

The pH of the bath of this invention may be in the range of about 1 to 6 and preferably 2 to 5. Generally a commercial bath will be operated at a pH of about 2.5 to about 4.5.

The temperature at which the plating process of this invention is carried out is not critical. Generally it is convenient to maintain temperatures in the range of from about 15°C to about 50°C and preferably from about 15°C to about 30°C.

Generally the anodes utilized with trivalent plating processes are carbon or graphite or other anode materials having a low overvoltage. These are referred to as inert anodes. Anode materials having a high overvoltage, generally insoluble metallic anodes such as lead, tend to assist oxidation of trivalent chromium ions to the undesirable hexavalent state and are generally not used. Similarly, soluble chromium anodes are generally not utilized.

### Example 1

A plating bath was prepared by dissolving the following materials in water and diluting to one liter:

The "chromium tanning salt" is chromic sulfate used in the tanning of leather, which is made by the reduction of sodium dichromate with sulfur dioxide. The material used has a "basicity" of 33%, basicity being a measure of the degree of replacement of sulfate ions by hydroxyl ions in the reduction product. The equilibrium pH of the bath after standing overnight was 3.4.

The bath prepared above was divided into two equal portions, Part A and Part B. To Part A was added 6 ml/I of a solution containing 100 g/I of potassium bromide, yielding a bromide concentration of 0.005 moles per liter in the bath. No bromide was added to Part B. The two solutions were placed in beakers equipped for magnetic stirring and circulatory cooling. Into each was inserted a carbon anode and a steel cathode, the anode to cathode area ration being 2:1. All electrodes were totally submerged in the baths. The two cells were connected in series with a source of direct current, and a current of 1.2 amps (2.4 amps/liter in each bath) was passed for one hour. The current densities were about 50 amps/ft² (ASF) (540 amps/m²) on the anodes and about 100 ASF (1100 amps/m²) on the cathodes.

The temperatures of both solutions were maintained between 25° and 27°C.

lnitially, Part A gave off a very mild odor, while the odor from Part B was strong. After 5 minutes the odor from Part B somewhat moderated, but the odor from Part A remaind much milder. For the remainder of the test period the intensity of odor from the two solutions varied, but that from Part A was always substantially lower than that from Part B.

### Example 2

A plating bath was formulated as follows:

The hydrochloric acid used was standard concentrated laboratory acid. The pH of the bath after equilibrating overnight was 3.4.

A sample of this bath was electrolyzed for 5 hours at 0.63 amp/liter, using a totally-submerged carbon anode at 50 ASF (540 amps/m²) and a totally-submerged steel cathode at 100 ASF (1100 amps/m²), The bath temperature was maintained between 17° and 22°C by the use of circulatory cooling during this operation. A highly objectionable odor was produced during this operation. A highly objectionable odor was produced continuously by the bath during plating.

An addition of solid potassium bromdie amounting to 0.89 g/I was made to this bath, giving a bromide ion concentration of 0.0075 mole per liter. The solution was air-agitated for 20 minutes, and the total anode and cathode areas were doubled. The current was started again, this time at 1.25 amps/I, but still maintaining 50 ASF (540 amps/m²) at the anode and 100 ASF (1100 amps/m²) at the cathode. It was found that the odor moderated to almost nothing within 4 minutes, and remained very slight after the passage of a total of 10 amp-hours/liter.

Comparison of plating tests run in the bath before and after the bromide ion addition and electrolysis showed that there was no effect on the cathode deposit, which was bright over a wide range of current density. The solution remained, at all times, free of hexavalent chromium, as shown by the plating results.

## Claims

1. A trivalent chromium plating bath comprising an aqueous solution of a trivalent chromium salt, at least one salt yielding chloride ion, at least one salt having a nitrogen-containing cation or substance yielding a nitrogen-containing cation and at least one salt yielding bromide ion, characterised in that the content of the bromide ion lies between 0.004 and 0.008 mole per liter.

2. A plating bath in accordance with Claim 1 further including at least one salt yielding sulfate ion in said bath.

3. A plating bath in accordance with Claim 1 or Claim 2, further including at least one of boric acid and borate ion.

4. A plating bath in accordance with any preceding claim, further including formate ion.

5. A process for producing a chromium containing electrodeposit comprising passing a current from an anode to a cathode through an aqueous solution including trivalent chromium ions, chloride ions, a nitrogen-containing cation and bromide ions for a period of time sufficient to form said electrodeposit characterised in that the bromide ion content lies between 0.004 and 0.008 mole per liter of the solution.

6. A process in accordance with Claim 5 wherein said anode is inert.

7. A process in accordance with Claim 6 wherein said anode is a carbon anode.

8. A process in accordance with any one of Claims 5 to 7 wherein the plating bath further includes sulfate ion.

9. A process in accordance with any one of Claims 5 to 8 wherein said bath further includes at least one of boric acid and borate ion.

10. A process in accordance with any one of Claims 5 to 9 wherein said bath further includes formate ion. 11. A process in accordance with any one of Claims 5 to 10 wherein the temperature is maintained in the range of about 15°C to about 50°C.

12. A process in accordance with any one of Claims 5 to 11 wherein the pH is maintained in the range of from about 1 to about 6.

## Patentansprüche

1. Ein dreiwertiges Chromplattierungsbad enthaltend eine wässerige Lösung eines dreiwertigen Chromsalzes, wenigstens eines Chloridionen abgebenden Salzes, wenigstens eines Salzes, das ein stickstoffhältiges Kation oder eine Substanz aufweist, die ein stickstoffhältiges Kation abgibt und wenigstens eines Salzes, das Bromidion abgibt, dadurch gekennzeichnet, daß der Gehalt an Bromidion zwischen 0,004 und 0,008 Mol/1 beträgt.

2. Ein Plattierungsbad nach Anspruch 1, weiters enthaltend wenigstens ein Salz, das Sulfation im genannten Bad abgibt.

3. Ein Plattierungsbad nach Anspruch 1 oder 2, weiters enthaltend wenigstens einen Bestandteil der Borsäure und Boration enthaltenden Gruppe.

4. Ein Plattierungsbad nach einem der vorhergehenden Ansprüche, weiters enthaltend Formiation.

5. Ein Verfahren zur Herstellung einer Chrom enthaltenden galvanischen Abscheidung umfassend das Durchleiten eines Stromes von einer Anode zu einer Kathode durch eine wässerige Lösung, die dreiwertige Chromionen, Chloridionen, ein stickstoffhältiges Kation und Bromidionen enthält, während eines Zeitraums, der ausreicht, um die genannte galvanische Abscheidung zu bilden, dadurch gekennzeichnet, daß der Bromidionengehalt zwischen 0,004 und 0,008 Mol/1 der Lösung beträgt.

6. Ein Verfahren nach Anspruch 5, worin die genannte Anode inert ist.

7. Ein Verfahren nach Anspruch 6, worin die genannte Anode ein Kohlenstoffanode ist.

8. Ein Verfahren nach einem der Ansprüche 5 bis 7, worin das Plattierungsbad weiters Sulfation enthält.

9. Ein Verfahren nach einem der Ansprüche 5 bis 8, worin das genannte Bad weiters wenigstens einen bestandteil der Borsäure und Boration enthaltenden Gruppe enthält.

10. Ein Verfahren nach einem der Ansprüche 5 bis 9, worin das genannte Bad weiters Formiation enthält.

11. Ein Verfahren nach einem der Ansprüche 5 bis 10, worin die Temperatur innerhalb eines bereiches von etwa 15°C bis etwa 50°C gehalten wird.

12. Ein Verfahren nach einem der Ansprüche 5 bis 11, worin der pH-Wert innerhalb eines Bereiches von etwa 1 bis etwa 6 gehalten wird.

## Revendications

1. Bain de placage à base de chrome trivalent comprenant une solution aqueuse d'un sel de chrome trivalent, au moins un sel donnant un ion chlorure, au moins un sel ayant un cation contenant de l'azote ou une substance donnant un cation contenant de l'azote et au moins un sel donnant l'ion bromure, caractérisé en ce que la teneur en ions bromurs est comprise entre 0,004 et 0,008 mole par litre.

2. Bain de placage selon la revendication 1 contenant de plus au moins un sel donnant l'ion sulfate dans ledit bain.

3. Bain de placage selon la revendication 1 ou la revendication 2, comprenant de plus au moins l'un parmi l'acide borique et l'ion borate.

4. Bain de placage selon l'une quelconque des revendications précédentes contenant de plus l'ion formiate.

5. Procédé de production d'un dépôt électrolytique contenant du chrome consistant à faire passer un courant d'une anode à une cathode à travers une solution aqueous contenant des ions de chrome trivalent, des ions chlorures, un cation contenant de l'azote et des ions bromure pendant un temps suffisant pour former ledit dépôt électrolytique, caractérisé en ce que la teneur en ions bromures est comprise entre 0,004 et 0,008 mole par litre de la solution.

6. Procédé selon la revendication 5 où l'anode précitée est inerte.

7. Procédé selon la revendication 6 où l'anode précitée une anode en carbone.

8. Procédé selon l'une quelconque des revendications 5 à 7 où le bain de placage contient de plus l'ion sulfate.

9. Procédé selon l'une quelconque des revendications 5 à 8 où ledit bain contient de plus au moins l'un de l'acide borique et de l'ion borate.

10. Procédé selon l'une quelconque des revendications 5 à 9 où ledit bain contient de plus l'ion formiate.

11. Procédé selon l'une quelconque des revendications 5 à 10 où la température est maintenue dans la plage d'environ 15°C à environ 50°C.

12. Procédé selon l'une quelconque des revendications 5 à 11 où le pH est maintenu dans la plage d'environ 1 à environ 6.
